

1

2,941,878

SOLID PROPELLENT COMPOSITIONS AND A  
PROCESS FOR THEIR PREPARATIONJohn E. Mahan and William M. Hutchinson, Bartlesville,  
Okla., assignors to Phillips Petroleum Company, a cor-  
poration of Delaware

No Drawing. Filed Jan. 27, 1956, Ser. No. 561,944

6 Claims. (Cl. 52—5)

This invention relates to improved solid propellant compositions and to a method for their preparation. In one of its aspects, this invention relates to novel solid propellant compositions having improved properties comprising an oxidant, a polymeric material and compounding ingredients therefor, and a burning catalyst.

Recently, it has been discovered that superior solid propellant materials are obtained comprising a solid oxidant such as ammonium nitrate or ammonium perchlorate, and a rubbery material such as a copolymer of butadiene and a vinylpyridine or other substituted heterocyclic nitrogen base compound, which after incorporation is cured by a quaternization reaction or a vulcanization reaction. Solid propellant mixtures of this nature and a process for their production are disclosed and claimed in copending application Serial No. 284,447, filed April 25, 1952, by W. B. Reynolds and J. E. Pritchard.

In the production of such solid propellant compositions, it is desirable that the products have good mechanical properties such as high elongation, low modulus, and high tensile strength as well as good burning rate.

It is an object of this invention to provide solid propellant compositions having a high value of elongation. It is also an object of this invention to provide solid propellant compositions having a low modulus of elasticity. It is also an object of this invention to provide a solid propellant composition having high tensile strength. It is a further object of this invention to provide a method for the production of solid propellant compositions having the above referred to properties of high elongation, low modulus of elasticity, and high tensile strength and also improved burning rate characteristics. It is an object to provide an improvement in properties of elongation and modulus in a propellant composition without sacrifice of properties of tensile strength. Other objects and advantages will be apparent to one skilled in this art upon study of the disclosure of this invention.

Broadly, the invention contemplates the preparation of a solid propellant composition comprising a solid oxidant and a binder comprising a rubbery copolymer of a conjugated diene and a heterocyclic nitrogen base and a minor portion of ammonium dichromate or a complex metal cyanide.

We have discovered that the addition of a minor portion of a complex metal cyanide or of ammonium dichromate to a propellant composition comprising a solid oxidant and a binder of a rubbery copolymer of a conjugated diene and a heterocyclic nitrogen base imparts a surprising increase in the rate of combustion of the propellant.

We have also discovered that solid propellant compositions comprising an ammonium nitrate-containing oxidant

2

and a binder comprising a rubbery copolymer of a conjugated diene and a heterocyclic nitrogen base can be improved in the properties of elongation and modulus of elasticity without a sacrifice of the property of tensile strength by incorporation therein, prior to curing, of a minor amount of ammonium dichromate or a complex metal cyanide such as milior blue, Prussian blue or Turnbull's blue. The specific beneficial results are obtained when the oxidant contains ammonium nitrate in an amount in excess of about 15 weight percent of the total oxidant.

The rubbery polymers employed as binders in the solid propellant compositions of this invention are copolymers of conjugated dienes with polymerizable heterocyclic nitrogen bases of the pyridine series. These copolymers can vary in consistency from very soft rubbers, i.e., materials which are soft at room temperature but will show retraction when relaxed, to those having a Mooney value (ML-4) up to 100. The rubbery copolymers most frequently preferred have Mooney values in the range between 10 and 40. They may be prepared by any polymerization methods known to the art, e.g., mass or emulsion polymerization. One convenient method for preparing these copolymers is by emulsion polymerization at temperatures in the range between 0 and 140° F. Recipes such as the iron pyrophosphate-hydroperoxide, either sugar-free or containing sugar, the sulfoxylate, and the persulfate recipes are among those which are applicable. It is advantageous to polymerize to high conversion as the unreacted vinylpyridine monomer is difficult to remove by stripping.

The conjugated dienes employed are those containing from 4 to 6 carbon atoms per molecule and include 1,3-butadiene, isoprene, 2-methyl-1,3-butadiene, 2,3-dimethyl-1,3-butadiene, and the like. Various alkoxy, such as methoxy and ethoxy and cyano derivatives of these conjugated dienes, are also applicable. Thus, other dienes, such as phenylbutadiene, 2,3-dimethyl-1,3-hexadiene, 2-methoxy-3-ethylbutadiene, 2-ethoxy-3-ethyl-1,3-hexadiene, 2-cyano-1,3-butadiene, are also applicable in the preparation of the polymeric binders of this invention. Instead of using a single conjugated diene, a mixture of conjugated dienes can be employed. Thus, a mixture of 1,3-butadiene and isoprene can be employed as the conjugated diene portion of the monomer system.

The polymerizable heterocyclic nitrogen bases which are applicable for the production of the polymeric materials are those of the pyridine, quinoline, and isoquinoline series which are copolymerizable with a conjugated diene and contain one, and only one,



substituent wherein R' is either hydrogen or a methyl group. That is, the substituent is either a vinyl or an alpha-methylvinyl (isopropenyl) group. Of these, the compounds of the pyridine series are of the greatest interest commercially at present. Various substituted derivatives are also applicable but the total number of carbon atoms in the groups attached to the carbon atoms of the heterocyclic nucleus should not be greater than 15 because the polymerization rate decreases somewhat with increasing size of the alkyl group. Compounds where the alkyl substituents are methyl and/or ethyl are available commercially.

These heterocyclic nitrogen bases have the formula



where R is selected from the group consisting of hydrogen, alkyl, vinyl, alpha-methylvinyl, alkoxy, halo, hydroxy, cyano, aryloxy, aryl, and combinations of these groups such as haloalkyl, alkylaryl, hydroxaryl, and the like; one and only one of said groups being selected from the group consisting of vinyl and alpha-methylvinyl; and the total number of carbon atoms in the nuclear substituted groups being not greater than 15. Examples of such compounds are 2-vinylpyridine; 2-vinyl-5-ethylpyridine; 2-methyl-5-vinylpyridine; 4-vinylpyridine; 2,3,4-trimethyl-5-vinylpyridine; 3,4,5,6-tetramethyl-2-vinylpyridine; 3-ethyl-5-vinylpyridine; 2,6-diethyl-4-vinylpyridine; 2-isopropyl-4-nonyl-5-vinylpyridine; 2-methyl-5-undecyl-3-vinylpyridine; 2,4-dimethyl-5,6-dipentyl-3-vinylpyridine; 2-decyl-5-(alpha-methylvinyl)pyridine; 2-vinyl-3-methyl-5-ethylpyridine; 2-methoxy-4-chloro-6-vinylpyridine; 3-vinyl-5-ethoxypyridine; 2-vinyl-4,5-dichloropyridine; 2-(alpha-methylvinyl)-4-hydroxy-6-cyanopyridine; 2-vinyl-4-phenoxy-5-methylpyridine; 2-cyano-5-(alpha-methylvinyl)pyridine; 3-vinyl-5-phenylpyridine; 2-(para-methylphenyl)-3-vinyl-4-methylpyridine; 3-vinyl-5-(hydroxyphenyl)-pyridine; 2-vinylquinoline; 2-vinyl-4-ethylquinoline; 3-vinyl-6,7-di-n-propylquinoline; 2-methyl-4-nonyl-6-vinylquinoline; 4-(alpha-methylvinyl)-8-dodecylquinoline; 3-vinylisoquinoline; 1,6-dimethyl-3-vinylisoquinoline; 2-vinyl-4-benzylquinoline; 3-vinyl-5-chloroethylquinoline; 3-vinyl-5,6-dichloroisoquinoline; 2-vinyl-6-ethoxy-7-methylquinoline; 3-vinyl-6-hydroxymethylisoquinoline; and the like.

Oxidants which are applicable in the solid propellant compositions of this invention include ammonium, alkali metal, and alkaline earth metal salts of nitric, perchloric, and chloric acids, and mixtures thereof. Ammonium nitrate and ammonium perchlorate are the preferred oxidants for use in the solid rocket fuels of this invention. Specific oxidants include sodium nitrate, potassium perchlorate, lithium chloride, calcium nitrate, barium perchlorate, and strontium chloride. Mixtures of oxidants are also applicable. In the preparation of the solid rocket propellant compositions, the oxidants are powdered to sizes preferably 300 to 10 microns average particle size. The amount of solid oxidant employed is usually a major amount of the total composition and is generally in the range between 50 and 90 percent by weight of the total mixture of oxidant and binder. If desired, however, less than 50 percent by weight of the oxidant can be used.

Combustion rate catalysts applicable in the invention include ammonium dichromate and metal ferrocyanides and ferricyanides. Ferric ferrocyanides, such as Prussian, Berlin, Hamburg, Chinese, Paris, and milori blue, soluble ferric ferrocyanide, such as soluble Berlin or Prussian blue which contains potassium ferric ferrocyanide, and ferric ferrocyanide which has been treated with ammonia, are among the materials which can be used. Ferrous ferricyanide, Turnbull's blue is also applicable. A particularly effective burning rate catalyst is milori blue which is pigment similar to Prussian blue but having a red tint and is prepared by the oxidation of a paste of potassium ferrocyanide and ferrous sulfate. Other metal compounds such as nickel and copper ferrocyanides can also be employed. The amount of burning rate catalyst used, in the propellant compositions of this invention, is usually in the range of 1 to 60 parts per one hundred

parts of rubbery polymer with from 5 to 50 parts being most frequently preferred. The amount of combustion catalyst will usually be 0.25 to 12 parts by weight per hundred parts of oxidant and binder.

The binder contains a rubbery copolymer of the type hereinbefore described and, in addition, there may be present one or more reinforcing agents, plasticizers, wetting agents, and antioxidants. Other ingredients which are employed for sulfur vulcanization include a vulcanization accelerator, a vulcanizing agent such as sulfur, and an accelerator activator, such as zinc oxide.

The copolymer comprising a conjugated diene and a polymerizable heterocyclic nitrogen base can also be cured by a quaternization reaction by incorporating thereinto a quaternizing agent and subjecting the resulting mixture to quaternizing conditions of temperature. Suitable quaternizing agents include alkyl halides such as methyl iodide, methyl bromide; alkylene halides such as methylene iodide, ethylene bromide; substituted alkanes such as chloroform, bromoform; alkyl sulfates such as methyl sulfate; and various substituted aromatic compounds such as benzoyl chloride, methyl benzene sulfonate, and the like.

The quaternizing temperature is usually in the range zero to 175° C., although temperatures outside this range can be used.

A general formulation for a binder composition prepared by sulfur vulcanization is given below:

|                                              | Parts by weight |
|----------------------------------------------|-----------------|
| Rubber copolymer (as hereinbefore described) | 100             |
| Reinforcing agent                            | 0-50            |
| Plasticizer                                  | 0-100           |
| Wetting agent                                | 0-10            |
| Antioxidant                                  | 0-3             |
| Vulcanization accelerator                    | 0-5             |
| Sulfur                                       | 0-2             |
| Zinc oxide                                   | 0-5             |

Reinforcing agents include carbon black, wood flour, lignin, and various reinforcing resins such as styrene-divinylbenzene, methyl acrylate-divinylbenzene, acrylic acid-styrene-divinylbenzene, and methyl acrylate-acrylic acid-divinylbenzene resins.

In general, any rubber plasticizers can be employed in these binder compositions. Materials such as Pentaryl A (amyl biphenyl), Parafflux (saturated polymerized hydrocarbon), Circosol-2XH (petroleum hydrocarbon softener having a specific gravity of 0.940 and a Saybolt Universal viscosity at 100° F. of about 2000 seconds), di(1,4,7-trioxaundecyl)methane, and dioctyl phthalate are suitable plasticizers. Materials which provide rubber having good low temperature properties are preferred. It is also frequently preferred that the plasticizers be oxygen-containing materials.

Wetting agents aid in deflocculating or dispersing the oxidizer, Aerosol OT (dioctyl ester of sodium succinic acid), lecithin, and Duomeen C diacetate (the diacetate of trimethylene diamine substituted by a coconut oil product) are among the materials which are applicable.

Antioxidants include Flexamine (physical mixture containing 25 percent of a complex diarylamine-ketone reaction product and 35 percent of N,N'-diphenyl-p-phenylenediamine), phenyl-beta-naphthylamine, 2,2-methylenebis(4-methyl-6-tert-butylphenol), and the like. Rubber antioxidants, in general, may be employed or if desired may be omitted.

Examples of vulcanization accelerators are those of the carbamate type, such as N,N'-dimethyl-S-tert-butylsulfenyl dithiocarbamate and Butyl-Eight. Butyl Eight is a rubber accelerator of the dithiocarbamate type supplied by the R. F. Vanderbilt Company and described in "Handbook of Material Trade Names" by Zimmerman and Lavine, 1953 Edition, as a brown liquid; specific gravity

1.01; partially soluble in water and gasoline; and soluble in acetone, alcohol, benzol, carbon disulfide and chloroform.

It is to be understood that each of the various types of compounding ingredients may be used singly or mixtures of various ingredients performing a certain function may be employed. It is sometimes preferred, for example to use mixtures of plasticizers rather than a single material.

The various ingredients in the propellant composition may be mixed on a roll mill or an internal mixer such as a Banbury or a Baker-Perkins dispersion blade mixer may be employed. The binder forms a continuous phase in the propellant with the oxidant as the discontinuous phase.

Rocket grains are formed by compression molding, injection molding, or extrusion.

The curing temperature will be limited by the oxidizer employed in some cases but will generally be in the range between 70 and 250° F., preferably between 170 and 200° F.

The curing time must be long enough to give required creep resistance and other mechanical properties in the propellant. The time will generally range from around three hours when the higher curing temperatures are employed to seven days when curing is effected at lower temperatures.

While this invention has been described using as the binder for propellant compositions a copolymer of a conjugated diene with a polymerizable heterocyclic nitrogen base of the pyridine series, such as vinylpyridine and various alkyl-substituted derivatives, it is to be understood that the corresponding quinoline and isoquinoline compounds are also applicable, i.e., vinylquinolines, vinylisoquinolines and various alkyl-substituted derivatives of these compounds.

#### EXAMPLE I

Two solid propellants were prepared having compositions as follows:

|                                             | Parts by Weight |    |
|---------------------------------------------|-----------------|----|
|                                             | 1               | 2  |
| Oxidizer (NH <sub>4</sub> NO <sub>3</sub> ) | 85              | 85 |
| Binder                                      | 15              | 15 |
| Milori blue                                 | 2               | 0  |

The binder composition was prepared using a 90/10 butadiene/2-methyl-5-vinylpyridine copolymer having a Mooney value (ML-4) of 20. This composition was prepared in accordance with the following formulation:

| Parts by weight                                   |      |  |
|---------------------------------------------------|------|--|
| Butadiene/2-methyl-5-vinylpyridine copolymer      | 100  |  |
| Carbon black                                      | 20   |  |
| Benzophenone                                      | 20   |  |
| N,N-dimethyl-S-tert-butylsulfenyl dithiocarbamate | 1    |  |
| Sulfur                                            | 0.75 |  |
| Zinc oxide                                        | 3    |  |
| Aerosol OT <sup>1</sup>                           | 1    |  |
| Flexamine <sup>2</sup>                            | 3    |  |

<sup>1</sup> Dioctyl ester of sodium sulfosuccinic acid.

<sup>2</sup> Physical mixture containing 25 percent of a complex diarylamine-ketone reaction product and 35 percent of N,N'-diphenyl-p-phenylenediamine.

The various ingredients making up the solid propellents were mixed in a Baker-Perkins dispersion blade mixer with the binder forming the continuous phase in the final composition. The material from each composition was extruded into strands  $\frac{3}{16}$  inches in diameter for ballistic test specimens and a sheet 0.25 inch in thickness from which tensile specimens were stamped out prior to curing. The specimens were cured 24 hours at 170° F. and mechanical and ballistic properties determined. Results are reported in the following Table I.

#### Table I

[Mechanical properties at 70° F., 3 in./sec. Cross Arm speed. Ballistic properties at 70° F., 1000 p.s.i.]

|                                   | 1     | 2      |
|-----------------------------------|-------|--------|
| 5                                 |       |        |
| Ultimate stress (tensile), p.s.i. | 335   | 264    |
| Ultimate elongation, percent      | 16.8  | 3.1    |
| Modulus of elasticity, p.s.i.     | 4,400 | 10,000 |
| Burning Rate, in./sec.            | 0.162 | 0.100  |
| n (pressure exponent)             | 0.53  | 0.65   |

10 <sup>1</sup> n is defined by the formula  

$$r = AP^n; \frac{r_1}{r_2} = \frac{AP_1^n}{AP_2^n}; r_1 = r_1 \frac{(P_1)^n}{(P_2)^n}; r = r_{1000} \frac{(P_1)^n}{(1000)^n}$$
  
<sup>2</sup> r=rate in./sec. at pressure P.  
<sup>3</sup> P=pressure of chamber p.s.i.g.  
<sup>4</sup> r<sub>1000</sub>=burning rate at the reference pressure of 1000 p.s.i.g.

#### EXAMPLE II

Two solid propellants having the following compositions were prepared:

|                                             | Parts by Weight |      |
|---------------------------------------------|-----------------|------|
|                                             | 1               | 2    |
| 20                                          |                 |      |
| Oxidizer (NH <sub>4</sub> NO <sub>3</sub> ) | 82.5            | 82.5 |
| Binder                                      | 17.5            | 17.5 |
| Milori blue                                 | 2               |      |
| Ammonium dichromate                         |                 | 2    |

30 The binder was prepared using a 90/10 butadiene/2-methyl-5-vinylpyridine copolymer having a Mooney value (ML-4) of 20. This composition was prepared in accordance with the following formulation:

|                                                   | Parts by weight |
|---------------------------------------------------|-----------------|
| 35 Butadiene/2-methyl-5-vinylpyridine copolymer   | 100             |
| Carbon black                                      | 20              |
| Benzophenone                                      | 10              |
| Pentaryl A                                        | 10              |
| N,N-dimethyl-S-tert-butylsulfenyl dithiocarbamate | 1               |
| Sulfur                                            | 0.75            |
| Zinc oxide                                        | 3               |
| Aerosol OT <sup>1</sup>                           | 1               |
| Flexamine <sup>1</sup>                            | 3               |

<sup>1</sup> As in Example I.

35 A Baker-Perkins dispersion blade mixer was employed for the mixing of various ingredients making up the solid propellant composition. The binder formed the continuous phase in the propellants. The material from each composition was extruded into strands  $\frac{3}{16}$  inch in diameter for ballistic test specimens and a sheet 0.25 inch in thickness from which tensile specimens were stamped out prior to curing. The specimens were cured 24 hours at 170° F. and mechanical and ballistic properties determined. The results are shown in Table II.

#### Table II

55 [Mechanical properties at 70° F., 3 in./sec. cross arm speed. Ballistic properties at 70° F., 1000 p.s.i.]

|                                      | 1     | 2     |
|--------------------------------------|-------|-------|
| 60 Ultimate stress (tensile), p.s.i. | 349   | 244   |
| Ultimate elongation, percent         | 19.5  | 29.5  |
| Modulus of elasticity, p.s.i.        | 4,300 | 2,945 |
| Burning Rate, in./sec.               | 0.182 | 0.177 |
| n (pressure exponent)                | 0.50  | 0.54  |

#### EXAMPLE III

65 Two solid propellants having the following compositions were prepared:

|                                             | Parts by Weight |      |
|---------------------------------------------|-----------------|------|
|                                             | 1               | 2    |
| 70                                          |                 |      |
| Oxidizer (NH <sub>4</sub> NO <sub>3</sub> ) | 82.5            | 82.5 |
| Binder                                      | 17.5            | 17.5 |
| Rouge                                       | 2               |      |
| Milori blue                                 |                 | 2    |

The binder was prepared using a 90/10 butadiene/2-methyl-5-vinylpyridine copolymer in accordance with the following formulation:

| Parts by weight                                       |      |
|-------------------------------------------------------|------|
| Butadiene/2-methyl-5-vinylpyridine copolymer          | 100  |
| Carbon black                                          | 20   |
| Benzophenone                                          | 10   |
| Pentaryl A (amylbiphenyl)                             | 10   |
| Butyl-Eight (dithiocarbamate-type rubber accelerator) | 2    |
| Sulfur                                                | 1.75 |
| Zinc oxide                                            | 3    |
| Aerosol OT <sup>1</sup>                               | 1    |
| Flexamine <sup>1</sup>                                | 3    |

<sup>1</sup> As in Example I.

The propellants were prepared as described in Examples I and II, and cured for 48 hours at 170° F. The results of tests are shown in Table III.

Table III

[Mechanical properties at 70° F., 3 in./sec. cross arm speed. Ballistic properties at 70° F., 1000 p.s.i.]

|                                   | 1     | 2     |
|-----------------------------------|-------|-------|
| Ultimate stress (tensile), p.s.i. | 322   | 340   |
| Ultimate elongation, percent      | 4.8   | 18.9  |
| Modulus of elasticity, p.s.i.     | 7,598 | 1,968 |
| Burning Rate, in./sec.            | 0.148 | 0.183 |
| n (pressure exponent)             | 0.57  | 0.59  |

#### EXAMPLE IV

The results of mechanical properties of Examples I, II, and III are compared in the following tabulation:

Table IV

| Propellant  | Catalyst, 2 parts by weight | Tensile, p.s.i. | Elongation, percent | Modulus, p.s.i. |
|-------------|-----------------------------|-----------------|---------------------|-----------------|
| Example I   | Milori blue                 | 335             | 15.8                | 4,400           |
| Example I   | None                        | 264             | 3.1                 | 10,000          |
| Example II  | Milori blue                 | 349             | 19.5                | 4,300           |
| Example II  | Ammonium dichromate         | 244             | 29.5                | 2,945           |
| Example III | Rouge                       | 322             | 4.8                 | 7,598           |
| Example III | Milori blue                 | 340             | 18.9                | 1,968           |

The binder formulations are not exactly the same in each case but the formulations are such as to provide a propellant in each case having an ultimate tensile strength in the range of 240 to 340 p.s.i. These tests demonstrate the advantages gained by the addition of milori blue or ammonium dichromate to the propellant formulation. In each case elongation values are higher and modulus values are lower than when rouge or no additive is used.

#### EXAMPLE V

A solid propellant was prepared having the following composition:

| Parts by weight                             |    |
|---------------------------------------------|----|
| Oxidizer (NH <sub>4</sub> NO <sub>3</sub> ) | 85 |
| Binder                                      | 15 |
| Milori blue                                 | 2  |

The binder was prepared using a 90/10 butadiene/2-methyl-5-vinylpyridine copolymer in accordance with the following formulation:

| Parts by weight                              |     |
|----------------------------------------------|-----|
| Butadiene/2-methyl-5-vinylpyridine copolymer | 100 |
| Carbon black                                 | 20  |
| Benzophenone                                 | 20  |
| Lauryl bromide                               | 14  |
| Flexamine <sup>1</sup>                       | 3   |

<sup>1</sup> As in Example I.

The propellant was prepared by thoroughly admixing the ingredients, shaping the mixture into the test pieces

and curing the specimens for 24 hours at 170° F. The results of tests with 3 in./min. cross-arm speed are as follows:

Table V

| Test Temperature, ° F. | Tensile, p.s.i. | Elongation, percent | Modulus, p.s.i. |
|------------------------|-----------------|---------------------|-----------------|
| 70                     | 198             | 15.1                | 2,126           |
| 170                    | 90              | 11.3                | 1,356           |
| 75                     | 863             | 15.0                | 7,128           |

This example shows that desirable values of elongation and modulus are obtained when quaternization is used to cure the propellant.

#### EXAMPLE VI

Five solid propellants were prepared having compositions as follows:

| Parts by weight                             |
|---------------------------------------------|
| Oxidizer (NH <sub>4</sub> NO <sub>3</sub> ) |
| Binder                                      |
| Milori blue                                 |

82.5

17.5

0, 0.25, 0.5, 1, 2

The binder composition was prepared using a 90/10 butadiene/2-methyl-5-vinylpyridine copolymer having a Mooney value (ML-4) of 20. The formulation employed for preparation of this composition was the same as that given in Example II.

The various ingredients making up the solid propellants were mixed on a roll mill. Tensile specimens from each composition were compression molded and burning rate strands were extruded. All specimens were cured 24 hours at 170° F. Results of burning rate tests at 70° F. and evaluation of mechanical properties on the propellants at 70° F. and 3 in./min. cross-arm speed are shown below:

35

Table VI

|                                               | 1      | 2     | 3     | 4     | 5     |
|-----------------------------------------------|--------|-------|-------|-------|-------|
| 40 Milori blue, parts                         | 0      | 0.25  | 0.5   | 1     | 2     |
| Strand burning rate at 1,000 p.s.i., in./sec. | 0.106  | 0.154 | 0.176 | 0.188 | 0.203 |
| Ultimate stress (tensile), p.s.i.             | 275    | 200   | 200   | 195   | 320   |
| Ultimate elongation, percent                  | 7      | 3     | 5     | 13    | 18    |
| Modulus of elasticity, p.s.i.                 | 12,500 | 8,500 | 7,000 | 4,000 | 5,000 |

45

The foregoing examples illustrate the unexpected improvement in the mechanical characteristics of the ammonium nitrate-containing propellant compositions where in milori blue or ammonium dichromate have been incorporated. Values of elongation are increased and values of modulus are decreased with no sacrifice of tensile strength values. It is noted that burning rate is progressively increased.

#### EXAMPLE VII

55 Solid propellants were prepared similar to those of the previous examples except that ammonium perchlorate was utilized as the oxidizer instead of ammonium nitrate. The binder compositions were as follows:

| Parts by weight |
|-----------------|
| 1               |
| 2               |
| 3               |
| 4               |
| 5               |

|                                                   |     |     |     |      |
|---------------------------------------------------|-----|-----|-----|------|
| 1-3-Butadiene/2-methyl-5-vinylpyridine copolymer  | 100 | 100 | 100 | 100  |
| Carbon black                                      | 22  | 22  | 22  | 22   |
| Butyl carbitol formal                             | 20  | 20  | 20  | 20   |
| N,N-dimethyl-S-tert-butylsulfonyl dithiocarbamate |     |     |     |      |
| Sulfur                                            |     |     |     | 0.75 |
| Zinc oxide                                        |     |     |     | 3    |
| Magnesium oxide                                   |     |     |     | 5    |
| Flexamine <sup>1</sup>                            | 3   | 3   | 3   | 3    |
| Benzotrichloride                                  | 6   | 6   | 6   | 6    |

Propellant compositions were as follows:

|                      |    |    |    |    |
|----------------------|----|----|----|----|
| Ammonium perchlorate | 85 | 85 | 85 | 85 |
| Binders (as above)   | 15 | 15 | 15 | 15 |
| Milori blue          | 2  | 2  | 2  | 2  |
| Ammonium dichromate  | 4  | 4  | 4  | 4  |

70

The propellants were prepared by thoroughly admixing the ingredients, shaping the mixture into test pieces and maintaining the specimens for 24 hours at 180° F. The results of tests are shown in the following Table VII.

Table VII

[Mechanical properties at 70° F., 2 in./min. cross-arm speed. Ballistic properties at 70° F., 1000 p.s.i.]

|                                        | 1     | 2     | 3     | 4        |
|----------------------------------------|-------|-------|-------|----------|
| Ultimate stress (tensile), p.s.i.----- | 180   | 129   | 164   | 26       |
| Ultimate elongation, percent.-----     | 15.9  | 11.3  | 9.1   | 46.4     |
| Modulus of elasticity, p.s.i.-----     | 1,720 | 1,850 | 2,430 | Very low |
| Burning rate, in./sec.-----            | 2.04  | 1.12  | 1.23  | 0.75     |
| <i>n</i> (pressure exponent)-----      | 0.51  | 0.45  | 0.45  | 0.22     |

The results of Example VII demonstrate the effect of incorporating a small amount of milori blue or ammonium dichromate in a solid propellant composition utilizing ammonium perchlorate as oxidant. The burning rate improvement is extremely high and provides a means for controlling the burning properties of a propellant composition.

Variations and modifications are possible within the scope of the disclosure of the present invention, the essence of which is the discovery that the addition of a minor amount of ammonium dichromate or a complex metal cyanide to a rocket propellant composition comprising a solid ammonium nitrate-containing oxidant, and a conjugated diene-heterocyclic nitrogen base copolymer provides an unexpected improvement in the mechanical characteristics of the propellant and in propellant compositions wherein ammonium nitrate is not employed in the oxidant a pronounced improvement in burning rate results from the presence of a minor amount of these materials.

That which is claimed is:

1. A propellant composition consisting essentially of an intimate admixture of from about 50 to about 90 parts by weight per 100 parts by weight of oxidizing salt and binder mixture of an inorganic oxidizing salt and from about 10 to about 50 parts by weight per 100 parts by weight of oxidizing salt and binder mixture of a binder selected from the group consisting of a sulfur vulcanized copolymer and a quaternized copolymer of (1) a conjugated diene having up to 8 carbon atoms per molecule; (2) at least one



substituted heterocyclic nitrogen base selected from the group consisting of pyridine, quinoline, alkyl substituted pyridine, and an alkyl substituted quinoline, wherein the total number of carbon atoms in the nuclear alkyl substituents is not more than 15 and wherein R' is selected from the group consisting of hydrogen and a methyl radical, 0 to about 50 parts by weight per 100 parts of copolymer of carbon black, 0 to about 100 parts by weight per 100 parts of copolymer of a rubber plasticizer, 0 to about 10 parts by weight per 100 parts of copolymer of an antioxidant, and 0 to about 3 parts by weight per 100 parts of copolymer of zinc oxide; and (3) about 0.25 to about 12 parts by weight per 100 parts of oxidizing salt and binder mixture of burning rate catalyst selected from the group consisting of ammonium dichromate and a complex cyanide of iron.

2. A composition of claim 1 wherein the inorganic oxidizing salt is ammonium nitrate; the conjugated diene is 1,3 - butadiene; the heterocyclic nitrogen base is 2-methyl-5-vinylpyridine; and the burning rate catalyst milori blue.

3. The composition of claim 1 wherein the inorganic oxidizing salt is ammonium nitrate; the conjugated diene

is 1,3 - butadiene; the heterocyclic nitrogen base is 2-methyl-5-vinylpyridine; and the burning rate catalyst is ammonium dichromate.

4. A propellant composition consisting essentially of from 50 to 90 parts by weight per 100 parts by weight of oxidizing salt and binder mixture of an inorganic oxidizing salt; from 10 to 50 parts by weight per 100 parts by weight of oxidizing salt and binder mixture of a binder consisting essentially of a copolymer of a conjugated diene having up to 8 carbon atoms per molecule and at least one



substituted heterocyclic nitrogen base selected from the group consisting of pyridine, quinoline, an alkyl substituted pyridine and an alkyl substituted quinoline, wherein the total number of carbon atoms in the nuclear alkyl substituents is not more than 15 and wherein R' is selected from the group consisting of hydrogen and a methyl radical, 0 to about 50 parts by weight per 100 parts of copolymer of carbon black, 0 to about 100 parts by weight per 100 parts of copolymer of a rubber plasticizer, 0 to about 10 parts by weight per 100 parts of copolymer of a wetting agent, and 0 to about 3 parts by weight per 100 parts of copolymer of an antioxidant; a curing amount of a curing agent selected from the group consisting of quaternization agents and sulfur vulcanization agents; and from 0.25 to 12 parts by weight of a burning rate catalyst; based on 100 parts by weight of oxidant-binder mixture, selected from the group consisting of ammonium dichromate and a complex cyanide of iron.

5. In a method for preparing a propellant composition which comprises forming an intimate admixture of 50 to 90 parts by weight per 100 parts by weight of oxidizing salt and binder mixture of an inorganic oxidizing salt; from 10 to 50 parts by weight per 100 parts by weight of oxidizing salt and binder mixture of a binder comprising a copolymer of a conjugated diene having up to 8 carbon atoms per molecule and at least one



substituted heterocyclic nitrogen base selected from the group consisting of pyridine, quinoline, an alkyl substituted pyridine and an alkyl substituted quinoline, wherein the total number of carbon atoms in the nuclear alkyl substituents is not more than 15 and wherein R' is selected from the group consisting of hydrogen and a methyl radical, and a curing amount of a curing agent selected from the group consisting of quaternization agents and sulfur vulcanization agents; the improvement comprising admixing with the aforesaid admixture from 0.25 to 12 parts by weight per 100 parts by weight of oxidizing salt and binder mixture of a burning rate catalyst selected from the group consisting of ammonium dichromate and a complex cyanide of iron; forming the mixture into grains; and curing the grains at a temperature in the range 70 to 250° F.

6. In a method for preparing a propellant composition which comprises forming a mixture consisting essentially of about 50 to about 90 parts by weight per 100 parts by weight of oxidizing salt and binder mixture of an inorganic oxidizing salt, about 10 to about 50 parts by weight per 100 parts by weight of oxidizing salt and binder mixture of a binder consisting essentially of a copolymer of a conjugated diene having up to 8 carbon atoms per molecule and at least one



substituted heterocyclic nitrogen base selected from the group consisting of pyridine, quinoline, an alkyl substituted pyridine and an alkyl substituted quinoline, wherein the total number of carbon atoms in the nuclear alkyl substituents is not more than 15 and wherein R' is selected from the group consisting of hydrogen and a

11

methyl radical, and sulfur vulcanization compounding ingredients and curing the resulting admixture at a temperature in the range of about 70 to about 250° F. to form a solid material, the improvement which comprises admixing about 0.25 to about 12 parts by weight per 100 parts by weight of oxidizing salt and binder mixture of a

12

burning rate catalyst selected from the group consisting of ammonium dichromate and a complex cyanide of iron with said oxidizing salt, copolymer and compounding ingredients prior to curing the said admixture to form said solid material.

5 No references cited.